

1

2,778,749

## PAPER PRODUCTS AND MANUFACTURE THEREOF

John P. Bainbridge, Jr., Marblehead, and Edward S. Blake, Lynnfield, Mass., assignors to Monsanto Chemical Company, St. Louis, Mo., a corporation of Delaware

No Drawing. Application December 22, 1952,  
Serial No. 327,448

19 Claims. (Cl. 117—154)

The present invention relates to paper articles and paper manufacture and it more particularly relates to the production of soft paper products, especially paper products of the facial tissue or other tissue type which are soft to the touch.

In preparing paper products suitable for use as paper toweling or facial tissue two methods of arriving at a product having satisfactory surface softness have been employed. In one of these methods the pulp used in preparing the tissue is beaten to such a slight degree that the paper formed therefrom has the requisite surface softness. Such products, however, have the disadvantage of being exceptionally weak and disintegrate readily to the annoyance of the user. In the other method the pulp used in preparing the tissue is beaten to such a degree that the paper formed therefrom will have a relatively satisfactory strength and will not disintegrate readily when used. However, such products per se are not sufficiently soft to the touch to be received favorably. In order to render such products commercially acceptable from the standpoint of surface softness, it is necessary to treat them with an agent which will give the requisite softness without introducing other objectionable features. Many chemical agents of the hygroscopic and waxy or wetting agent type have been tried for this purpose. A few have been successful to a limited extent but they do not give the optimum surface softness desired. Many agents have been tried unsuccessfully and these have been unsuccessful for various reasons. One primary reason for failure is that they do not impart the requisite surface softness to paper. Some agents accomplish this in some degree but they introduce complicating factors such as bad odor, poor aging properties, toxic effects, decreased water absorbency, etc. For example, glycerine which is a hygroscopic agent, gives a softening effect but has the disadvantage of lowering the tensile strength and the water absorbency of the tissue, and it also imparts an objectionable damp feel to the tissue. As another example, sodium oleate, which is a wetting agent, has the disadvantages of poor aging characteristics and insufficient softening action. Many other examples of specific agents which have been found to be unsuitable could be cited but it is believed the remarks made with respect to the agents specifically mentioned indicate that the suitability of any particular agent for the surface softening of paper facial tissue cannot be predicted.

It is one object of this invention to provide methods for softening the surface of paper products.

It is a further object of this invention to provide paper products which are softer to the touch than the paper per se.

It is a further object of this invention to provide paper suitable for use as facial tissue and having the requisite surface softness and utility for such purpose.

Still further objects and advantages of this invention will become apparent from the following description and the appended claims.

2

The objects of this invention are attained, in general, by providing a paper product, preferably paper facial tissue, containing a water soluble aliphatic disulfonic acid containing at least 10 carbon atoms or water soluble derivatives thereof in an amount sufficient to soften the paper product but insufficient to impair the utility of such paper product.

The aliphatic disulfonic acid containing at least 10 carbon atoms or water soluble derivatives thereof, hereinafter referred to as the agent for convenience in description, may be applied directly to the paper after it is formed or it may be incorporated into the paper product prior to the manufacture of such product on the paper machine. The first of these procedures is preferred since it provides a paper product of higher tensile strength and does not interfere with the manufacturing process for producing the paper product. A particularly preferred method of application comprises spraying an aqueous solution of the agent on the surface or surfaces of the paper product which it is desired to soften. For example, if the paper is in the form of a sheet and it is only desired to soften one surface of the sheet, the agent need only be applied to that surface.

The solution of the agent is most suitably applied by spraying the solution on the paper product since this procedure does not appreciably affect the wet or dry tensile strength of the product. However, when the lowering of the wet or dry tensile strength of the paper product is not undesirable, the solution of the agent may be applied to the paper product in other ways. To obtain a uniform softening effect, the agent should be applied uniformly to the paper product. In applying the agent to the paper product by spraying, it is preferred to adjust the spray and the solids concentration of the agent in solution so as to obtain little or no surface wetting of the paper product. Under such conditions the agent is deposited primarily on the surface of the paper product and appreciable penetration of the agent into the body of the paper product is avoided, and no marked change in the properties of the paper product, other than softening of the surface to the touch, is noted.

The agent may also be incorporated in the paper product by adding it to a paper furnish, that is, an aqueous slurry of paper pulp from which the paper sheet or product is produced. However, this procedure does not give as good a result as the procedure of applying the agent to the paper product since the addition of the agent to the furnish results in foaming and other operating difficulties during the paper forming process and the strength of the product is less than when the agent is not added to the furnish.

The agent may be applied to or incorporated in any paper product where softness or lack of harshness to the touch is desirable or required, for example, creped or uncreped sanitary tissues, facial tissues, toilet tissues, toweling and the like. Such products are usually prepared from unsized to lightly sized pulps such as bleached or unbleached sulfite, sulfate, soda or groundwood pulps or mixtures of such pulps. The present invention is particularly directed to the softening of paper products which are used on the human skin and where softness to the touch, non-toxicity, non-irritation and satisfactory strength of the product are essential properties. The agents of this invention are most suitably applied to such paper products as have a satisfactory strength for their intended use but do not per se have the requisite surface softness.

The amount of agent used on or in the paper product may be varied considerably depending primarily on the particular agent used, the intended use of the paper product and the type of pulp from which the paper product is manufactured. However, normally the agent

is used in small amounts, with some surface softening being obtained in most cases by the application of as little as 0.05% by weight of the agent, based on the dry weight of the paper product. However, in order to obtain a considerable surface softening effect, it is preferable to apply at least 0.1% by weight of the agent, based on the dry paper product. Ordinarily, no advantages accrue in applying more than 2% by weight of the agent, based on the dry paper product, and it is preferred, in order to avoid alteration of the paper product properties, to apply not more than 1% by weight of the agent, based on the dry paper product. In general, therefore, the agent is applied to or incorporated in the paper products in amounts of about 0.05 to 2% by weight, and preferably between 0.1 and 1% by weight, based on the dry paper product.

The agents employed in this invention comprise the class of compounds which include the aliphatic disulfonic acids which consist of a normal or branched saturated carbon chain having from 10 to 30 carbon atoms to which are attached hydrogen atoms and two sulfonic acid groups ( $-\text{SO}_3\text{H}$  groups), or halogenated derivatives thereof containing up to two halogen atoms, preferably chlorine atoms, attached to a carbon atom or atoms, or water-soluble salts of such compounds including the ammonium and alkali metal mono- or di-salts. The alkali metal salts, particularly the di-sodium salts, are preferred over the acids per se or other water-soluble salts. The position occupied by the sulfonic acid groups or halogen, if such latter group is present, on the carbon chain is apparently not critical. As examples of compounds which may be employed may be mentioned dodecane disulfonic acids, dichloro dodecane disulfonic acids or the mono- or di-sodium salts of such acids; cetane disulfonic acids or the mono- or di-sodium salt thereof; octadecane disulfonic acids or mono-chlor octadecane disulfonic acids or the mono- or di-sodium salts of such acids; eicosane disulfonic acids or the mono- or di-sodium salt thereof; and the like. The preferred compounds from the standpoint of number of carbon atoms are those which contain from 16 to 22 carbon atoms.

The disulfonic acids employed in this invention and described above may be prepared by first reacting 1 mol of an alkane containing at least 10 carbon atoms, for example, from 10 to 30 carbon atoms, and preferably from 16 to 22 carbon atoms, with 2 mols of sulfur dioxide ( $\text{SO}_2$ ) and 2 mols of chlorine (2  $\text{Cl}_2$ ) in the presence of ultra-violet light at a temperature between about 35 and 80° C. until the alkane contains two sulfo-chloride ( $\text{SO}_2\text{Cl}$ ) groups, after which the product is hydrolyzed with an alkanol to form the disulfonic acid and the corresponding chloride of the alcohol or is hydrolyzed with an alkali metal hydroxide to form the corresponding disulfonic acid and alkali metal chloride. After separation of the disulfonic acid and alkyl chloride as, for example, by distillation of the alkyl chloride from the product, the disulfonic acid may be employed as such or neutralized with a base capable of forming a water-soluble mono- or di-salt of such acid. Ammonium and alkali metal hydroxides or carbonates may be used for this purpose.

The agents employed in this invention are preferably soluble or dispersible in water to the extent of at least 25% by weight, and more particularly to the extent of about 25 to 60% by weight.

A further understanding of the processes and products of this invention will be obtained from the following specific examples which are intended to illustrate this invention but not to limit the scope thereof, parts and percentages being by weight.

#### Example I

A 50% aqueous solution of the disodium salt of a dodecane disulfonic acid was sprayed uniformly on both sides of a creped, unsized paper facial tissue of double

thickness in an amount sufficient to deposit 0.5% of such salt on the tissue surface, based on the dry tissue weight. The tissue was then supercalendered. Whereas the original tissue, prior to treatment, had satisfactory strength and resistance to disintegration when wet, such tissue was not sufficiently soft to be commercially acceptable. The treated tissue, on the other hand, not only possessed the strength and resistance to disintegration of the original tissue, but was sufficiently soft to be commercially acceptable. Moreover, the treated tissue was non-toxic, was free of objectionable odor or color and did not acquire a bad odor or color over long periods of aging.

#### Example II

15 A 50% aqueous solution of the disodium salt of an eicosane disulfonic acid was applied to both sides of a creped, unsized paper facial tissue of double thickness according to the procedure of Example I. The treated tissue was then supercalendered and was found to be 20 softer than the treated tissue of Example I, but was otherwise equivalent in properties.

Similar results were obtained with the disodium salt of a mono-chlor eicosane disulfonic acid and with an eicosane disulfonic acid, with the exception that the latter 25 compound rendered the tissue acidic.

Various changes and modifications may be made in the processes and paper products described herein, as will be apparent to those skilled in the art to which this invention appertains, without departing from the spirit and 30 intent of this invention. Accordingly, it is to be understood that it is not intended to limit this invention except by the scope of the appended claims.

What is claimed is:

35 1. A cellulosic fiber paper product comprising a substance selected from the class consisting of aliphatic disulfonic acids having at least 10 carbon atoms, halogen-containing aliphatic disulfonic acids having at least 10 carbon atoms and containing up to 2 halogen atoms which are attached to a carbon atom of said acid and water-soluble salts of said compounds, said substance being present in an amount sufficient to soften the surface of 40 said paper product.

2. A cellulosic fiber paper product comprising an aliphatic disulfonic acid having from 10 to 30 carbon atoms, 45 said acid being present in an amount sufficient to soften the surface of said paper product.

3. A cellulosic fiber paper product as in claim 2, but further characterized in that said acid is present in amounts of about 0.05 to 2% by weight based on the dry paper 50 product.

4. A cellulosic fiber paper product comprising a chlorinated aliphatic disulfonic acid having from 10 to 30 carbon atoms and up to two chlorine atoms which are attached to a carbon atom of said acid, said substance being present in an amount sufficient to soften the surface of said paper product.

5. A cellulosic fiber paper product comprising a water-soluble salt of a chlorinated aliphatic disulfonic acid having from 10 to 30 carbon atoms and up to two chlorine atoms which are attached to a carbon atom of said acid, said substance being present in an amount sufficient to soften the surface of said paper product.

6. A cellulosic fiber paper product comprising a water-soluble salt of an aliphatic disulfonic acid having from 65 10 to 30 carbon atoms, said salt being present in an amount sufficient to soften the surface of said paper product.

7. A cellulosic fiber paper product as in claim 6, but further characterized in that said salt is a sodium salt.

8. A cellulosic fiber paper product for use on human skin comprising a sodium salt of an aliphatic disulfonic acid having from 10 to 30 carbon atoms, said salt being present on the surface of said product which contacts the skin in an amount sufficient to soften said product to the 75 touch.

9. A cellulosic fiber paper product as in claim 8, but further characterized in that the paper product is selected from the class consisting of facial tissues, sanitary tissues, toilet tissues and paper toweling.

10. A cellulosic fiber paper product as in claim 9, but further characterized in that said salt is present in amounts of from about 0.1 to 1% by weight based on the dry paper product.

11. A cellulosic fiber paper product as in claim 8, but further characterized in that the compound is a sodium salt of an aliphatic disulfonic acid having from 16 to 22 carbon atoms.

12. A process of softening cellulosic fiber paper products which comprises applying to said products an aqueous solution of a substance selected from the class consisting of aliphatic disulfonic acids having at least 10 carbon atoms, halogen-containing aliphatic disulfonic acids having at least 10 carbon atoms and containing up to 2 halogen atoms which are attached to a carbon atom of said acid and water-soluble salts of said compounds, said substance being applied to said product in an amount sufficient to soften the surface of said product, and allowing said paper product to dry.

13. A process of softening cellulosic fiber paper products which comprises spraying on said products an aqueous solution of at least 25% by weight of an alkali metal salt of an aliphatic disulfonic acid having from 10 to 30 carbon atoms, said solution being sprayed in an amount sufficient to deposit from 0.05 to 2% by weight of said salt, based on the dry paper product, and allowing said paper product to dry.

14. A process as in claim 13, but further characterized in that said paper products are selected from the class consisting of sanitary tissues, facial tissues, toilet tissues and paper toweling.

15. A process as in claim 14, but further characterized in that said alkali metal salt is a sodium salt.

16. A process of softening cellulosic fiber paper facial tissue which comprises spraying on said tissue an aqueous solution of at least 25% by weight of a sodium salt of an aliphatic disulfonic acid having from 16 to 22 carbon atoms, said solution being sprayed on the outer surface of said tissue without appreciably wetting said tissue and in an amount sufficient to deposit from about 0.1 to 1% by weight of said salt, based on the dry weight of said tissue, and allowing said tissue to dry.

17. A process as in claim 16, but further characterized in that said aliphatic disulfonic acid is an eicosane disulfonic acid.

18. A process as in claim 17, but further characterized in that said salt is the disodium salt.

19. A process of producing soft cellulosic fiber paper products which comprises adding a substance selected from the class consisting of aliphatic disulfonic acids having at least 10 carbon atoms, halogenated derivatives of said acids containing up to 2 halogen atoms which are attached to a carbon atom of said acid and water-soluble salts of said compounds to an aqueous slurry of paper pulp, forming the paper pulp into a paper product and thereafter drying said paper product, said substance being present in an amount sufficient to soften the surface of the paper product prepared from said paper pulp.

References Cited in the file of this patent

UNITED STATES PATENTS

|    |           |         |       |               |
|----|-----------|---------|-------|---------------|
| 30 | 1,986,291 | Schur   | ----- | Jan. 1, 1935  |
|    | 2,032,645 | Youtz   | ----- | Mar. 3, 1936  |
|    | 2,061,619 | Downing | ----- | Nov. 24, 1936 |
|    | 2,412,909 | Potter  | ----- | Dec. 17, 1946 |

FOREIGN PATENTS

|         |               |       |               |
|---------|---------------|-------|---------------|
| 280,262 | Great Britain | ----- | Nov. 15, 1927 |
| 534,618 | Great Britain | ----- | Mar. 12, 1941 |